

April 6, 1937.

H. S. GEORGE

2,075,810

BUILT-UP RAIL AND METHOD OF BUILDING UP THE SAME

Filed Sept. 6, 1933

2 Sheets-Sheet 1



INVENTOR  
**HARRY S. GEORGE**  
BY  
*E. Greenwald*  
ATTORNEY

April 6, 1937.

H. S. GEORGE

2,075,810

BUILT-UP RAIL AND METHOD OF BUILDING UP THE SAME

Filed Sept. 6, 1933

2 Sheets-Sheet 2



INVENTOR  
HARRY S. GEORGE  
BY *E. Greenwald*  
ATTORNEY

## UNITED STATES PATENT OFFICE

2,075,810

BUILT-UP RAIL AND METHOD OF BUILDING  
UP THE SAMEHarry S. George, Massapequa, N. Y., assignor, by  
mesne assignments, to Union Carbide and Car-  
bon Corporation, a corporation of New York

Application September 6, 1933, Serial No. 688,333

24 Claims. (Cl. 29—169)

This invention relates to rails having built-up tread surface areas, and to a method of building them.

The tread surfaces at the ends of rails at joints in track become battered to a lower level than the rest of the tread surfaces of rails, because at the ends of rails there is no support against end flow of rail metal at the tread surfaces thereof; hence, the rate at which tread surfaces of rails become battered is greatest at rail ends. This lowering of the running or tread surfaces of rails at rail joints increases the effect of the pressure of rolling traffic by converting it into a downward blow as the wheels pass over rail joints. This action still further increases the rate at which the tread surfaces at the ends of rails become battered over that of the rest of the rails. After a few years of service the amount of batter at rail joints becomes so great that, in order to increase the life of rails, the battered tread surfaces at the ends of rails are built-up to the general level of the rails by depositing metal on the depressed areas.

In order to facilitate an understanding of this invention, it seems expedient at the outset to consider the manner in which metal deposited on the battered or worn tread surface areas of rails cools and hardens. The metal generally deposited is a steel, and, generally speaking, the more rapidly steel cools the greater its hardness becomes. After a depressed worn tread surface area of a rail is built-up by depositing the metal thereon at an elevated temperature, as by welding, the cooling from such elevated temperature of the metal deposited and the rail metal adjacent thereto is chiefly brought about naturally by the conduction of heat into the rail itself. It is to be understood that the expression "natural cooling" signifies the combined cooling effect of convection and radiation of heat from the rail to the surrounding air plus the cooling effect of the underlying and adjacent mass of the rail which is relatively cool. I have found that the latter effect is much greater than the cooling effect of air where a relatively small tread surface in an ordinary rail is heated, as in the case of building up the tread surfaces at the ends of rails.

From an observation of the performance of built-up rails under modern traffic conditions, I have discovered that built-up tread surface areas at the extreme ends of rails at joints should possess a hardness of at least 60 Scleroscope after being subjected to service if they are to withstand the tendency to flow. In order to attain this

hardness, the metal must have a Scleroscope hardness of about 50 to 52 after it is deposited and before the metal is subjected to service, the Scleroscope hardness increasing with service or cold work, as it is commonly called. The Scleroscope hardness of about 50 to 52 corresponds to a Brinell hardness of about 350. It has been found that the increase in hardness due to cold work is generally not indicated by the Brinell test, and hence the Brinell value of hardness remains substantially the same before and after service.

It has generally been the practice heretofore to build up worn areas on rail heads in one continuous operation, as by progressively depositing the metal thereon. With rails of the size now generally used, such as rails weighing 100 to 130 pounds per yard, it is possible to attain the desired hardness mentioned above at rail ends and tread surface areas intermediate the ends of rails when worn areas approximately up to three inches in length and of average depth of wear are built up in one continuous operation with suitable weld metal, such as weld metal of the composition hereinafter described. In such cases natural cooling is sufficiently rapid to produce built-up rail tread surface areas having a hardness of at least 50 to 52 Scleroscope before service and a hardness of at least 60 Scleroscope after service.

The tread surfaces of modern rails now supplied to railroad companies possess a hardness of about 250 to 275 Brinell. This hardness is less than that required to prevent the flow of tread surface metal at the ends of rails. Although weld metal of the character hereinafter described is capable of possessing a hardness sufficient to prevent flow of rail tread surface metal, such hardness is not attained when it is deposited by prior methods, as just described.

The desired hardness is not uniformly attained, however, where longer worn areas, such as areas of more than three inches in length having an average depth of wear, are built up in one continuous operation; or where short areas of about three inches in length having an excessive depth of wear are built up in a similar manner in the tread surfaces of tracks. This is particularly true at the tread surfaces at rail ends where it has been found that the metal deposited at the "run off" zone or the portion adjacent to the unworn tread surface of the rail is considerably harder than the metal deposited at the "end zone" or the portion adjacent to the extreme end of the rail head. With prior methods not only is the "end zone" 55

the softest part of the built-up rail head, but it does not possess sufficient hardness to withstand the pounding and hammering of rolling traffic. Tests of built-up rails of the type just described 5 indicate that only the portion of the deposit adjacent to the unworn tread surface attains the desired hardness mentioned above. This is due to the fact that the metal at the "run off" zone of the deposit is adjacent to the unheated part of 10 the rail and will cool more rapidly than the metal at the "end zone", which is away from the unheated part of the rail. Stated another way, the heat input is greater with a larger deposit and the rate of cooling of the portion near the ex- 15 treme end of the rail head is dependent upon the relatively cool mass at the end of the rail where the heat applied tends to be concentrated. The mass of the rail back from the end thereof is considerably cooler, because there is no tendency of 20 the heat to be concentrated. Hence, the con- 25 duction of heat from the metal deposited on the rail head is faster at the portion adjacent to the unworn tread surface of the rail.

In addition to the manner in which the metal 25 deposited cools and hardens, other factors that affect the rate of cooling are the size of the rail, the size of the worn area, and the temperature of the rail, which, in turn, is dependent upon the heat input required for depositing the metal on a 30 worn area of a rail head. Laboratory tests indicate that none of the above factors can be controlled enough to sufficiently increase the hardness when a worn area on a rail head is built-up in one continuous operation. In other words, 35 long deposits of metal of the character above described cannot be made fast enough on worn tread surface areas to insure a minimum hardness at the extreme end of the rail head of about 50 Scleroscope before service, even when the partic- 40 ular operator, such as a welder, is highly skilled.

Building up worn areas of rail tread surfaces in this manner is objectionable, because it is desired that the metal deposited be of sufficient and adequate hardness at the extreme end of the rail 45 head where the tendency of the metal deposited to wear and flow is severest. Further, such built-up rails are lacking in uniformity as to thickness, composition and hardness of the metal deposited, primarily because of the differences of skill of the 50 individual operators in depositing the metal on the worn areas of rails.

As far as is known, no successful method of building up worn tread surface areas of rails has been devised to overcome the objections mentioned 55 above. For example, in Railway Engineering and Maintenance, February, 1933, it is stated on page 76 that the greater hardness of metal deposited on worn tread surface areas at the "run-off" zone, as compared with the lower hardness thereof at 60 the "end zone", cannot be overcome.

I have found that the difficulties previously encountered in building up worn tread surface areas of rails can be overcome by what I term the "interrupted" method. In this method metal is de- 65 posited only on a portion of a worn area and cooled. Subsequently, after the metal first deposited has cooled, metal is deposited on another portion of the worn tread surface area and cooled. In carrying out my "interrupted" method of building 70 up worn tread surface areas of rails in practice, the metal deposited on each portion of a worn tread surface area is preferably hardened entirely by natural cooling, without employing any external quenching medium to assist in the cool- 75 ing and hardening of the metal deposited on the

rail head. In this preferred method of building up worn tread surface areas of rail, the metal deposited on each portion of a worn area is allowed to cool sufficiently before metal is deposited on another portion, so as not to render ineffective the natural cooling and hardening of the metal that is deposited on each succeeding portion. In this manner metal deposits of adequate hardness can be produced on worn areas of rail heads by an operator of average skill, irrespective of the length or depth of the deposit. Further, by the interrupted method, the required hardness can be imparted to the deposited metal, such as metal of the character hereinafter described, which is potentially capable of being so hardened. 15

I have also found that the relatively large worn areas at ends of rails now generally encountered in practice can be avoided by forming a much smaller built up tread surface area at the ends of rails when they are new and before they are subjected to service. 20

An object of this invention, therefore, is to provide rails having steel or alloy steel deposited on worn tread surface areas thereof which hardens sufficiently so that it will not wear and flow away when subjected to service. 25

Another object of my invention is to provide such rails having built-up tread surface areas at the ends thereof in which the metal deposited possesses a hardness of at least 350 Brinell before service at the portions where the tendency of the metal to wear and flow is greatest. 30

A further object of my invention is to provide such rails having built-up tread surface areas in which at least portions of the metal deposited possess adequate hardness to withstand wearing and flowing and are of such shape that they are utilized most effectively when subjected to traffic. 35

A further object of my invention is to provide an "interrupted" method of building up worn tread surface areas of rails uniformly whereby the differences of skill of the individual operators, such as welders, in depositing the metal on the worn areas, is substantially eliminated. 40

A further object of my invention is to provide an improved method of building up worn tread surface areas of rails in which the rate of natural cooling of the metal deposited can be controlled. 45

A further object of my invention is to provide an improved method of building up worn tread surface areas of rails whereby a portion of the metal deposited on a worn area is reheated and hardened to a higher degree than before with the subsequent depositing of metal on another portion of the worn area adjacent to the metal previously deposited. 50

A further object is to provide a method of building up tread surface areas of new rails or rails not subjected to service whereby the life 60 of rails is prolonged and track maintenance is reduced considerably.

Further objects and advantages of my invention will become apparent as the following description proceeds, and the various features of 65 novelty which characterize my invention are pointed out with particularity in the claims annexed to and forming a part of this specification. In the drawings:

Fig. 1 is a plan view of a typical rail joint 70 showing the battered areas before the rails are built up;

Fig. 2 is a side view of the rail joint shown in Fig. 1;

Figs. 3, 4 and 5 are plan views of rail joints, 75

similar to the joint shown in Figs. 1 and 2, built up in accordance with the principles of this invention; and

Fig. 6 is an explanatory diagram showing the hardness at different points of the rail joint illustrated in Fig. 1 when built up by my improved method.

In Fig. 1 is illustrated diagrammatically the approximate shape of the battered areas 10 and 11 of a typical worn rail joint formed by aligned rails 12 and 13 having an opening 14 therebetween. This figure represents an open joint of a straight and level track on which the traffic is unidirectional or "one-way" in the direction 15 indicated by the arrow. The average depth of batter or wear normally encountered in practice varies from approximately .02 to .06 inches at the extreme ends of the heads of the rails, and this distance, which is purposely exaggerated, is indicated at 15 between the arrowed lines in Fig. 2. In order to illustrate one particular application of building up rails by my improved "interrupted" method, it will be assumed that the worn tread surface area 10 on "leaving" rail 12 extends back 25 approximately three inches from the extreme end of the rail 12; that the worn tread surface area 11 on "receiving" rail 13 extends back approximately five inches from the extreme end of the rail 13; and that the weight of the rails is about 30 130 pounds per linear yard. The above assumptions closely approximate actual track conditions.

Since the worn tread surface area 10 is assumed to be approximately three inches in 35 length in the particular embodiment which has been chosen to illustrate the principles of this invention, it is possible to attain the desired hardness when metal is deposited thereon in one continuous operation, because natural cooling 40 will be sufficiently rapid to effect the proper rate of cooling of the metal deposited. The desired hardness is not attained, however, when the metal is deposited in one continuous operation on worn tread surface area 11, because the rate 45 of cooling will not be sufficiently rapid, especially at the extreme end of the head of the rail 13.

The desired degree of hardness can be attained, however, when the worn tread surface area 11 is built up by my "interrupted" method. In 50 accordance with this improved method, metal is deposited on the entire worn area 11 except a portion at the extreme end of the rail head; and, subsequently, after an interruption to allow the rail to cool, metal is deposited on the remaining 55 portion of the worn tread surface area 11 at the extreme end of the rail head.

This "interrupted" method of building up rail ends may be accomplished in practice in several different ways. When the worn tread surface 60 areas at each rail joint are to be built up at the same time, the "interrupted" method may be carried out in the following manner.

Referring to Fig. 3, only the portion 16 of the worn tread surface area 11, which is shaded by 65 solid lines, is built up first by depositing metal directly on the head of the rail. The depositing of metal on the worn area 11 is then interrupted to allow the metal deposited to harden with natural cooling. In order to utilize effectively the 70 time during this interruption in building up worn tread surface area 11, the entire worn tread surface area 10, which is shaded by dotted lines, may be built up by depositing metal on the head of the rail. When natural cooling is employed 75 the operator generally can start to de-

posit metal directly on the rail head at the portion 17 of the worn area 11, which is shown by solid cross hatching, immediately after the worn area 10 has been built up. The metal should be deposited on the portion 17 of the worn tread surface area 11 so that it will form a sound and firm deposit at the extreme end of the rail head, and so that it will unite thoroughly with the metal previously deposited on the rail head at the portion 16. To insure hardening of the metal 10 deposited on the portion 17 with natural cooling, the metal first deposited on the portion 16 should be allowed to cool to at least a black heat. A considerable increase in hardness is obtained 15 when the metal first deposited only on the portion 16 is allowed to cool to atmospheric temperature before any metal whatsoever is deposited on portion 17.

When a considerable number of successive joints in an entire section of track are to be 20 built up, the following procedure, which effectively economizes time, has been carried out in practice in building up depressed tread surfaces at rail ends by the "interrupted" method: Each 25 operator, such as a welder, is assigned ten successive rail joints along a section of track. The portions 16 of the worn tread surface areas 11 and the worn tread surface areas 10 are first built up successively on all ten joints. Afterwards 30 the operator builds up the portions 17 of the worn areas 11 successively on all ten joints in the same order as the building up previously done. In this manner the interruption in building up the worn areas 11 is sufficiently long to 35 allow the metal first deposited on the rail head only at the portion 16 to cool nearly to atmospheric temperature before metal is deposited on the rail heads at the portions 17.

In building up rails by the "interrupted" method, two factors that influence the hardness of 40 the metal deposited on the tread surface at the extreme end of the rail 13 are the size of the rail and the area of the portion 17. Generally, the larger the size of the rail the greater is the 45 rate of natural cooling. As shown in Fig. 4, 50 the size of the portion 17' of the worn area 11' is considerably smaller than the portion 17 shown in Fig. 3. One reason for such a smaller portion 55 17' may be that the rails 12' and 13' are of smaller weight than the rails 12 and 13; and another reason may be that it is desired to obtain an increased hardness of the metal deposited on the tread surface at the extreme end of the rail head by effecting a more rapid rate of 60 natural cooling.

When open rail joints of the type illustrated in 65 Figs. 3 and 4 are built up by my "interrupted" method, some consideration should be given to the manner in which the welding heat is applied when metal is deposited on the rail heads at 70 the portions 17 and 17', so that there will be no tendency for the hardness to be drawn from the previously built-up areas 10 and 10'. In building up the last portions 17 and 17', the welding heat for depositing metal on the rail 75 heads may be applied in such a manner that a minimum amount of heat is applied to the adjacent areas 10 and 10', so that the hardness of the metal previously deposited on the rail heads at the areas 10 and 10' will remain substantially unchanged. This particular manner of building up worn tread surface areas of rails has been successfully carried out in practice.

In certain instances, particularly where the opening in a joint is relatively small, the oper- 75

ator or welder in building up the portions 17 and 17' may apply the welding heat for depositing metal on the rail heads in such a manner that the extreme end portions of the metal deposited on the areas 18 and 18' are reheated to at least a hardening heat. These end portions of deposited metal which are reheated are preferably of the same size and shape as the portions 17 and 17' which are built up last, so as not to attain too great a hardness of the portions of metal which are reheated. With this procedure a high degree of hardness of the metal deposited on the rail heads at the portions 17 and 17' is attained, and at the same time the end portions of the metal deposited on the worn tread surface areas 10 and 10' will harden with natural cooling.

In order to assist in preventing the drawing of the hardness of the metal deposited on the worn tread surface area at the extreme end of one rail at a rail joint when metal is to be deposited on a worn tread surface area at the extreme end of the abutting rail, it may be desirable in certain instances to arrange a metallic block over the worn area first built up to shield the metal deposited thereon from the welding heat which is applied on the rail head of the abutting rail when the worn tread surface area at the end thereof is built up. For example, in the present instance it may be desirable to arrange a copper block over the built-up areas 10 and 10' to aid in preventing the drawing of the hardness of the metal deposited when welding heat is applied on the heads of rails 18 and 18' for depositing metal thereon at the portions 17 and 17'.

The mass of the copper block should be sufficiently large so that it will stand up during the application of heat when the last portions of the depressed surfaces of rail heads are built up, and is preferably of U-shape so that the side walls thereof will extend downward over the sides of the rail head and rest on the angle bars so as to support the block in position. An end wall or fin may be provided for further protection at one end of the U-shaped block, which end wall is adapted to extend downward into the opening between the ends of the abutting rails of a joint. The block is preferably made of copper because of its high heat capacity and conductivity so as to prevent any melting thereof on the rail tread surface while exposed to the heat which is applied on the rail.

In certain instances, as where the rail joints are so close together that the metal deposited on abutting worn areas bridges over the ends of the aligned rails, the "interrupted" method of building up tread surface areas of rails at rail joints is slightly modified. In Fig. 5 is illustrated a rail joint comprising aligned rails 12" and 18" abutting each other. In this modified method metal is first deposited on the heads of rails 12" and 18" only at the portion 18" of the worn area 11" and the portion 18" of the worn area 10". The depositing of metal is then interrupted, and, after the metal deposited has cooled, metal is deposited in one continuous operation on the rail heads at the remaining portions 17" and 18" of the worn areas 10" and 11".

In the typical rail joint illustrated in Figs. 3 and 4, the "interrupted" method of building up a worn tread surface area at a rail end has been shown as applied to the worn area at the end of the "receiving" rail in a section of track in which the traffic is one way or unidirectional.

In such cases the end of the "receiving" rail generally has the largest worn area. When the worn tread surface areas at both rail ends at a rail joint are of such length that the desired hardness is not attained by building them up continuously in one operation, as in a section of track where the traffic moves in both directions, each worn area of a rail joint may be built up by the "interrupted" method. Also, the end of the "leaving" rail may have a worn tread surface area more than three inches in length in certain instances, and in such cases the worn area at the end of the "leaving" rail is built up by the "interrupted" method.

As will be noticed in Fig. 1, the shapes of the worn tread surface areas are such that the inside edges 20 and 21 of the rail heads are worn a greater distance back from the extreme ends of the rails 12 and 18 than the outside edges 22 and 23 of the rail heads. This is due to the fact that, as the wheels of rolling stock move over a straight track in which the rails are usually only slightly canted, the tires of the wheels bear on the middle portion of the tread surfaces and inside edges of the rail heads. The wearing and flowing of rail metal starts at the ends and inside edges of the heads of the rails 12 and 18, and gradually works back from the ends of the rail heads. After considerable wearing and flowing, the depressed worn areas 10 and 11 are produced which slope downward and toward the inside edges 20 and 21 of the rail heads. The greatest flowing and wearing of the metal at rail ends, therefore, occurs at the extreme ends of the rail heads, the inside edges of the rail heads, and the inside and middle portions of the tread surfaces of the rails.

Taking into consideration the manner in which traffic tends to cause deformation or wear at the ends of rail heads in straight track, I preferably build up worn tread surface areas of rails by the "interrupted" method so that the last portions built up, such as the portion 17, extend a longer distance back from the ends of the rails on the inside edges than on the outside edges of the rail heads. In cases where rails are canted a considerable amount and where track maintenance is such that the greatest wear occurs from the middle to the outside edges of rail heads, the last portions can be preferably built up so that they extend a longer distance back from the ends of the rails on the outside edges than on the inside edges of the rail heads. In this manner the portions of tread surfaces of rail heads having the greatest tendency to wear when subjected to traffic are included in the last portion on which metal is deposited.

In order to attain an adequate degree of hardness of the metal deposited on rail heads at the extreme ends of rails, it is desirable that the last portions built up be not unduly large, so that a rapid rate of natural cooling is effected. For this reason I prefer to make the last portions built up of approximately trapezoidal shape, as shown in Fig. 3, or of approximately triangular shape, as shown in Figs. 4 and 5, because for a sufficiently rapid rate of cooling to insure adequate hardness of the metal deposited, they are the smallest areas which will also give sufficient length longitudinally of the rail in such a manner that the areas are effectively utilized to prevent wearing and flowing of the metal deposited on the tread surfaces at the ends of rails.

Where the tread surface at the end of a rail

head is not worn away at its outside edge, the last portion built up need not extend across the entire width of the rail head, as illustrated by the portion 17' in Fig. 4, for example.

5 The metal having a greater alloy content than that of the rail metal may be deposited on the rail heads at the worn tread surface areas either by gas, by electric welding, or by any other suitable source of high temperature heat. I preferably build up rails by gas welding with a suitable combustible gas, such as a mixture of oxygen and acetylene. A hardenable steel I prefer to deposit on worn areas of rail heads contains approximately .50% carbon, 0.90 to 1.10% manganese, 0.90 to 1.10% chromium, 0.40 to 0.60% silicon and the remainder iron. However, any suitable steel or alloy steel having characteristics similar to the composition of steel just mentioned can be used that is capable of hardening when cooled from an elevated temperature.

20 Before the metal is welded on the worn areas of rail heads by the "interrupted" method, any chips or cracks requiring an abnormal amount of welding are preferably built up first to the general level of the battered area. Also, if the depth of a battered or worn area is less than .04 to .06 of an inch, additional rail metal may be removed if desired, as by grinding or with a welding torch, so that all built-up rails will have a deposit of 25 appreciable depth after leveling and smoothening by grinding.

25 I prefer to use a gas flame or flames as the source of high temperature heat for depositing a hardenable metal on worn tread surface areas, and for this purpose a suitable burner, such as a blowpipe, may be employed. The burner may be supplied with a suitable combustible gas, such as a mixture of oxygen and acetylene. When building up rail tread surfaces by depositing a 30 hardenable metal thereon with an oxy-acetylene flame, a strictly neutral flame can be used. Since frequent adjustments may be necessary to maintain a neutral flame, an excess acetylene flame having a "feather" of excess acetylene of about 35 two to three times the length of the inner cone is preferred because of the protection of the rail metal and metal deposited from oxidation. Further, an excess acetylene flame tends to carburize the surface of the rail metal and superficially melt it by the formation of a high-carbon-iron alloy having a melting point below that of the rail steel. This superficial melting, or "wetting" 40 or "sweating" as it is sometimes termed, is an aid in insuring a perfect union between the metal deposited and the rail metal. Since there is a 45 continuous tendency for rail metal at the tread surface to be chilled by the withdrawal of heat therefrom by the relatively cool mass of the rail, it is desirable for the less skillful welder, when 50 using an excess acetylene flame, to melt into the rail tread surface slightly below the "wet" film while depositing metal, so as to insure good fusion 55 of the metal deposited and rail metal.

55 In welding metal to the first portion of a battered area of a rail head, such as the portion 18, it is preferable in the present instance to deposit the metal last at the inside edge of the tread surface to insure a maximum hardness at the flange or inside edge of a rail head, which is 60 subjected to greater wear than the outside edge of the rail head. The metal is preferably deposited on the tread surface portions at the extreme end of the rail, such as the portion 17, from the inside edge to the outside edge of the rail head, and the welding should be such that

65 the metal last deposited on the rail head is thoroughly welded both to the adjacent underlying rail metal and to the metal first deposited and back from the extreme end of the rail. The welding of metal on the portion of the tread surface 70 at the extreme ends of rail heads should be continuous, so that the entire portion last built up cools as a unit from an elevated hardening temperature to insure built-up rails of uniform and sufficient hardness. The metal last deposited 75 should of course not be reheated after it has once cooled. Any welding or shaping of its surface or edges should be done before it has cooled below the hardening temperature.

80 Not only is the metal last deposited on the extreme ends of rail heads cooled and hardened to a high degree in the manner described above, but part of the metal first deposited on rail heads back from the extreme ends of rails is rehardened to a higher degree than before, because of the heat applied on the metal first deposited when metal is deposited on rail heads at the extreme ends of the rails. In other words, when the metal last deposited on the rail head is welded to the edge of the metal first deposited 85 on the rail head, a portion of the metal first deposited is reheated to an elevated hardening temperature. This reheated metal cools naturally with the metal last deposited at the extreme end of rail heads, and its degree of hardness is increased considerably. This is an important advantage of the "interrupted" method of building up rails, because the relatively harder portions of built-up tread surface areas at the extreme ends of rail heads are increased in size.

90 By making the portions of worn areas last built up of substantially triangular or trapezoidal shape, the junction or boundary between such built-up portions and the portions first built up extends approximately diagonally across the tread surfaces of rails. This is of considerable importance as the metal last deposited on a portion of a worn tread surface area is considerably harder than the metal first deposited 95 on another portion of the worn area, and by extending the boundary therebetween along the longitudinal direction of the rail head, a diagonal run-off is provided whereby the wheels of rolling stock at no point of their travel have to pass immediately over tread surface metal of one hardness onto tread surface metal of a considerably 100 different hardness.

105 In Fig. 6 is shown an explanatory diagram indicating the hardness, after being subjected to service, of the built-up ends of rails of the rail joint illustrated in Fig. 3, in which the weight of the rails is about 130 pounds per linear yard, the length of the worn tread surface area at the end of the "receiving" rail is approximately five 110 inches long, and the length of the worn tread surface area at the end of the "leaving" rail is approximately three inches long. The irregular lines 24 and 25 indicate the hardness produced of the metal deposits at different points of such a joint by an operator or welder above average skill. At the end of the "leaving" rail, where the metal is deposited continuously on the rail head, it will be noticed that the maximum hardness at 115 the end of the rail head at A is about 66 Scleroscope after service or cold work, and remains at 120 a hardness above 60 Scleroscope for approximately the full length of the deposit. At the end of the "receiving" rail, where the metal is deposited by the "interrupted" method, it will be noticed that the hardness of the metal deposit 125

is adequate to withstand wearing and flowing for at least a distance of 2 inches from the extreme end of the rail head, varying between 68 and 71 Scleroscope at the points B and C. This distance not only represents the portion of the metal deposited last, but also a part of the portion of the metal deposited first which is rehardened to a higher degree than before, when the last portion of the worn area is built up at the extreme end 10 of the rail head. The hardness of the metal first deposited is lower than that at the extreme end of the rail, increasing from 58 Scleroscope at D to about 60 Scleroscope at E, which is adjacent to the unworn tread surface of the "receiving" 15 rail. At the point F is indicated the hardness of the unworn rail metal adjacent to the built-up area at the end of the rail.

In order to emphasize the advantage of building up worn tread surface areas of rails by the 20 "interrupted" method, so as to produce a metal deposit having adequate hardness at the portion of the worn tread surface area adjacent to the extreme end of the rail, the portion E—D of the irregular line 25 has been extended as a dotted 25 line to the point G, to indicate the relative hardness of a metal deposit built up by the continuous method. It will be noticed that, with such a method of building up worn tread surface areas of rails, the deposit is softest at the extreme end 30 of the rail head and of a hardness below that which will withstand deformation and wear. Irregular lines 24' and 25', similar to lines 24 and 25, indicate the hardness attained of the metal deposits at different points of a joint by an operator or welder of average skill. In such cases, 35 the hardness at A' is about 61 Scleroscope, the hardness between B' and C' varies from 62 to 65 Scleroscope, and the hardness between D' and E' varies from about 55 to 58 Scleroscope. The 40 lower relative hardness of a metal deposit built up by the continuous method is indicated by the dotted line between D' and G'.

It will thus be seen that, when worn tread surface areas of rails are built up by the "interrupted" method, built-up rails are produced having a hardness of at least 60 Scleroscope after 45 cold work or service at the extreme ends of the rail heads, and that this hardness is produced by an operator or welder of average skill as well 50 as an operator above average skill. In order to produce built-up rail tread surface areas along a section of track which are of substantially uniform hardness, the size of the portion of the worn tread surface area last built up can be 55 determined to suit the natural speed and habit of each operator or welder. Thus, if an operator of average skill can produce built-up worn tread surface areas of the desired hardness with the last portion of the worn area of a given size, the 60 size of the last portion built up can be increased for an operator above average skill. In this manner the rate of natural cooling, and hence 65 the hardness produced of the metal deposited, can be controlled and made substantially uniform for all operators.

In the explanatory diagram just described, the 70 different values of hardness given are those attained when the metal deposited is of the composition mentioned above. It is to be understood that the composition of the metal deposit is somewhat different from that of the metal supplied, as there is some loss of metal in slagging and some of the metal deposited mixes with 75 the rail metal, which, together with the effect

of the flame, will slightly increase the carbon content of the metal deposited. However, by depositing metal in the manner indicated above, a considerable amount of hardening material remains in the built-up deposit.

The values of hardness attained will vary slightly, of course, with differences in the hardening ability of the metal deposited on rail heads, the size of the last portion of the worn tread surface area which is built up, and other factors, such as the particular composition of the rail steel and the welding technique; but with due regard for these factors, worn tread surface areas can be built up by the "interrupted" method so that the metal last deposited on a portion of a worn area will be of adequate and sufficient hardness to withstand wearing and flowing.

The relatively large worn areas now generally encountered in practice can be avoided by building up portions of tread surfaces when rails are new and before they are subjected to service. Thus wearing and flowing of rail tread surface metal which normally occurs is anticipated, thereby prolonging the life of rails from the very beginning and reducing track maintenance considerably. This is particularly true at the ends of rail tread surfaces, although in many instances it is applicable to tread surface areas intermediate to the ends of the rails.

In building up tread surface areas at the ends of unworn rails, the original rail metal on the top of the rail head is removed in any suitable manner, as by machining, grinding, or with a welding torch. The original rail metal is removed to a sufficient depth, such as .04 to .16 of an inch, for example, so that the metal deposited will be of appreciable depth after leveling and smoothening by grinding. A suitable metal, such as the hardenable metal of the composition mentioned above, having adequate hardness to withstand wearing and flowing when subjected to service is then deposited on the tread surface area to build the same up to the general level of the rail. Since such a tread surface area is generally relatively small, it may be possible and 35 preferable to deposit the metal in one continuous operation, and to limit the size of the area in accordance with the principles employed in the "interrupted" method, so as to control the hardness of the deposited metal between maximum and minimum limits. The built up tread surface area may then be leveled and smoothened by grinding. At rail ends the build-up areas are preferably triangular or trapezoidal in shape 40 because, as stated before, it is the smallest area which will give sufficient length longitudinally of the rail in such a manner that the area is effectively utilized to prevent wearing and flowing of rail metal. By building up small tread surface areas on the top surfaces of rail heads in 45 the manner just described, considerably larger worn areas are avoided. For example, if the end of the rail 13 in Fig. 3 had been built up before being subjected to service so that the built-up area only constituted the portion 17, the much 50 larger worn area 11 would have been avoided.

Throughout the specification a distinction has been made in Scleroscope hardness before and after service. While a definite relation exists between Brinell and Scleroscope hardness for 55 the same metal, this relation is not the same for a thin alloy deposit, or for a rail that has been in service and has a cold worked surface. It has been found that hardening due to cold work further tends to prevent flow of the metal de- 60

posed, and therefore constitutes a beneficial or protective action.

As a result of considerable experience, it has been found that the Brinell test is not suitable for testing the hardness of rails having a thin surface layer whose hardness is different from that of the underlying metal. It has been found that the increase in hardness due to cold work is not fully indicated by the Brinell test, where-  
10 as such increase in hardness is indicated by the Scleroscope test. For the above reasons, the Brinell hardness is compared with the Scleroscope hardness before the metal tested is subjected to cold work, and a different Scleroscope hardness is indicated for metal after cold work.

From an observation of the performance of rail ends, it has been stated above that a Brinell hardness of about 350 and a Scleroscope hardness of about 50 to 52 before service and 60 after 20 service is adequate to prevent flow of the metal deposited. There is no objection to an even greater hardness, such as a hardness of 70 Scleroscope after service, if the deposit is sound and tough and not accompanied by brittleness 25 and heat cracks. In view of the foregoing, it will be apparent that by the interrupted method of building up rail tread surfaces the hardness at the deposited metal acquired can be controlled, especially at the extreme ends of the 30 rails; and this control of hardness is such as to insure the attainment of not only the minimum hardness required to prevent flow of tread surface metal, but also to insure that the hardness does not exceed any desired maximum value, 35 thereby obviating the occurrence of cracks in the deposited metal.

While I have shown and described built-up rails and a method of building them up by the "interrupted" method with a single interruption, 40 it will be obvious that battered or worn tread surface areas of rails can be built up by depositing metal on rail heads and interrupting the depositing of such metal on several successive portions of a worn area, and that the "interrupted" method can be employed in building up worn tread surface areas at points intermediate the ends of rails as well as at the ends of rails. It is to be understood that new or unworn and 45 worn rails can be built up by the methods described either with gas flames or the electric arc, and that modified methods of producing built-up rails having a hardness of at least 60 Scleroscope will occur to those skilled in the art without departing from the spirit and scope of my invention.

I claim:

1. A rail having at an end thereof a built-up tread surface portion comprising metal having an alloy content greater than that of the 50 rail metal, such portion being more than three inches in length longitudinally of the rail and having adjacent the extreme end of the rail a hardness of at least 60 Scleroscope after cold rolling, said portion being of such shape that at 55 least a part of the boundary between said built-up portion and the portion of the rail tread surface adjacent thereto extends approximately diagonally across the rail tread surface.

2. A rail having at an end thereof a built-up 60 tread surface portion comprising metal having an alloy content greater than that of the tread surface metal adjacent thereto, such portion being more than three inches in length longitudinally of the rail and having adjacent the 65 extreme end of the rail a hardness of at least

60 Scleroscope after cold rolling, said built-up tread surface portion at the extreme end of the rail being of such shape that it extends back from the end of the rail a greater distance at one edge than the other edge of the rail head. 5

3. A method of improving substantially unworn rails having a tread surface portion at an end thereof tending to wear and flow when subjected to service, which comprises removing a surface layer of original rail metal at such 10 a tread surface portion, the length of such layer longitudinally of the rail being less than about three inches, and subsequently depositing thereon before the rail is subjected to service a metal capable of acquiring a hardness of at least 60 15 Scleroscope after cold rolling.

4. A method of improving substantially unworn rails having a tread surface portion of an end thereof tending to wear and flow when subjected to service, which comprises removing a 20 surface layer of original rail metal at such a tread surface portion, the length of such portion longitudinally of the rail being less than about three inches; and subsequently depositing thereon, before the rail is subjected to service, a metal 25 capable of acquiring a hardness of at least 60 Scleroscope after cold rolling, the layer of deposited metal being of such shape that the boundary between said deposited metal and the portions of the rail tread surface adjacent thereto extends diagonally across the rail tread surface. 30

5. A method of increasing the wearing characteristics of the tread surface areas at the ends of substantially unworn rails, which comprises 35 removing a surface layer of original rail metal at such a tread surface area, the length of such layer longitudinally of the rail being less than about three inches, and subsequently depositing thereon before the rail is subjected to service 40 a metal capable of acquiring a hardness of at least 60 Scleroscope after cold rolling, the shape 45 of the area formed by the metal deposited being such that it extends back from the end of the rail a greater distance at one edge than the other edge of the rail head.

6. A rail having at an end thereof a built-up tread surface portion comprising metal having an alloy content greater than that of the rail metal, such portion being more than about three 50 inches in length longitudinally of the rail and having the greatest hardness at the portion adjacent to the end of the rail head.

7. A rail having at an end thereof a built-up tread surface area portion comprising metal having an alloy content greater than that of the rail metal, such portion being more than three inches in length longitudinally of the rail and having the greatest hardness at the portion adjacent to the extreme end of the rail head, such portion 60 adjacent to the extreme end of the rail head having a hardness of at least 60 Scleroscope after cold rolling.

8. A method of building up a depressed tread surface at the end of a rail which comprises first welding a layer of metal to the major portion of said surface but not to a portion of the surface adjacent to the end of the rail, and welding additional metal to the portion of the surface adjacent to the end of the rail after the first-welded 65 layer has cooled.

9. A method of building up a depressed tread surface of a rail in which a steel capable of hardening upon cooling from an elevated temperature is deposited on such surface by welding; such 75

method comprising depositing the steel by welding on one portion of the surface and subsequently depositing the steel successively to other portions of the surface so that the steel deposited on each portion joins the steel previously deposited to form an integral deposit; the steel deposited and rail metal adjacent thereto always being sufficiently cool so as not to render ineffective the quenching effect produced by the mass of the rail on the steel deposited on each succeeding portion and the rail metal adjacent thereto, whereby welding heat is withdrawn from the steel welded to each succeeding portion to cool and harden the same naturally.

15 10. A method of building up a depressed tread surface of a rail in which a steel capable of hardening upon cooling from an elevated temperature is deposited on such surface by welding; said method comprising welding the steel on one portion of the surface and subsequently welding the steel to the remaining portion of the surface; the steel welded to the first portion of the surface and the rail metal adjacent thereto being sufficiently cool before the steel is welded to the remaining portion of the surface so as to render effective the quenching effect produced by the mass of the rail on the steel welded to the remaining portion of the surface and rail metal adjacent thereto, whereby welding heat is withdrawn from the steel welded to the remaining portion of the surface to cool and harden the same naturally.

11. A method of building up a depressed tread surface of a rail in which a steel capable of hardening upon cooling from an elevated temperature is deposited on such surface by welding; said method comprising depositing the steel by welding on a portion of the surface; and thereafter, after such deposited steel and rail metal adjacent thereto have cooled to at least a black heat, depositing the steel by welding to another portion of the surface so that the steel subsequently deposited joins the steel previously deposited to form an integral deposit.

45 12. A method of building up a depressed tread surface of a rail in which a steel capable of hardening upon cooling from an elevated temperature is deposited on such surface by welding; said method comprising depositing the steel by welding to one portion of the surface; and thereafter, after such deposited steel and rail metal adjacent thereto have cooled to at least a black heat, depositing the steel by welding to the remaining portion of the surface.

55 13. A method of building up a worn tread surface at the end of a rail in which a steel capable of hardening upon cooling from an elevated temperature is deposited on such surface by welding; said method comprising depositing the steel by welding to the entire worn surface except a portion at the extreme end of the rail head; interrupting the depositing of the steel; and subsequently depositing the steel by welding to the portion of the surface at the extreme end of the rail head; said interruption being of such duration that the steel deposited first and rail metal adjacent thereto are sufficiently cool to render effective the quenching effect produced by the mass of the rail on the steel deposited on the portion at the extreme end of the rail head and the rail metal adjacent thereto, whereby welding heat is withdrawn from the steel deposited on the portion at the extreme end of the rail head to cool and harden the same.

75 14. A method of building up a depressed tread

surface at the end of a rail in which a steel capable of hardening upon cooling from an elevated temperature is deposited on such surface by welding; said method comprising depositing the steel by welding to the entire surface except a portion at the extreme end of the rail head; interrupting the depositing of the steel; and subsequently depositing the steel by welding to the portion of the surface at the extreme end of the rail head; the steel being so deposited on the first portion that at least a portion of the boundary between the steel deposited first and the steel subsequently deposited at the extreme end of the rail head extends approximately diagonally across the rail tread surface; said interruption being of such duration that the steel deposited first and rail metal adjacent thereto are sufficiently cool to render effective the quenching effect produced by the mass of the rail on the steel deposited at the extreme end of the rail head and the rail metal adjacent thereto, whereby welding heat is withdrawn from the steel deposited on the portion at the extreme end of the rail to cool and harden the same.

15 15. A method of building up a depressed tread surface at the end of a rail in which a steel capable of hardening upon cooling from an elevated temperature is deposited on such surface by welding; said method comprising depositing the steel by welding on the entire surface except a portion at the extreme end of the rail head; interrupting the depositing of steel until the steel deposited and rail metal adjacent thereto have cooled to at least a black heat; and subsequently depositing the steel by welding to the portion of the surface at the extreme end of the rail head.

20 16. A method of building up a worn tread surface area at the end of a rail in which a steel capable of hardening upon cooling from an elevated temperature is deposited on such surface by welding; said method comprising depositing the steel by welding on the entire worn surface except a portion at the extreme end of the rail head; interrupting the depositing of steel until the steel deposited and rail metal adjacent thereto have cooled to at least a black heat; and subsequently depositing the steel by welding to the portion of the surface at the extreme end of the rail head; the steel being so deposited on the first portion that at least a portion of the boundary between the steel deposited first and the steel subsequently deposited at the extreme end of the rail head extends approximately diagonally across the rail tread surface.

25 17. A self-hardening method of building up a depressed tread surface of a rail in which a metal capable of hardening upon cooling from an elevated temperature is deposited on such surface by welding; said method comprising depositing the metal successively on several portions of the surface and allowing the metal deposited on each portion to cool naturally before the metal is deposited on a succeeding portion.

30 18. A self-hardening method of building up a depressed tread surface of a rail in which a metal capable of hardening upon cooling from an elevated temperature is deposited on such area by welding; such method comprising depositing the metal on one portion of the surface and allowing the same to cool naturally; and subsequently depositing the metal on the remaining portion of the surface and allowing the same to cool naturally.

35 19. A method of building up a worn rail joint

comprising abutting rails having depressed tread surfaces at the ends thereof, one of such depressed surfaces being larger than the other; said method comprising first welding metal on such surfaces but not the portion at the end of the rail head having the largest depressed surface; and subsequently welding the metal on the portion of the surface at the end of the rail having the largest depressed area after the first-  
10 welded metal has cooled.

20. A method of building up a worn rail joint comprising abutting rails having depressed tread surfaces at the ends thereof; said method comprising first welding metal on such surfaces but not the portions at the end of the rails; and subsequently welding metal on the portions of the depressed surfaces at the ends of the rails after the first-welded metal has cooled.

21. A rail having at an end thereof a built-up tread surface area comprising metal having an alloy content greater than that of the rail metal, the portion of such area adjacent to the extreme end of the rail head having a greater hardness than the portion back from the extreme end of the rail head, the shape of the portions being such that at least a part of the boundary therebetween extends approximately diagonally across the rail tread surface.

22. A rail having at an end thereof a built-up tread surface area comprising metal having an alloy content greater than that of the rail metal, the portion of such area adjacent to the extreme end of the rail head having a greater hardness than the portion back from the extreme end of the rail head, the shape of the portion adjacent to the extreme end of the rail head being such that it extends a greater distance back from the extreme end of the rail head at 10 one edge of the rail than at the other edge thereof.

23. A rail having adjacent an end thereof a built-up top tread surface portion comprising fusion-deposited metal having a greater hardness than the rail metal, said built-up portion being of such shape that at least a sufficient portion of its boundary distant from the end of the rail extends diagonally across the rail tread surface to provide a diagonal run-off which will 20 prevent rolling stock from passing abruptly from the harder built-up portion to the adjoining tread surface.

24. A rail as claimed in claim 23, in which the distance of said boundary from the end of the rail is greatest adjacent the inner edge of said tread surface.

HARRY S. GEORGE.